

# UNITED STATES PATENT OFFICE.

JAMES TAYLOR, OF ANSONIA, CONNECTICUT, ASSIGNOR TO THE ELECTRICAL SUPPLY COMPANY, OF SAME PLACE.

## COATING AND INSULATING WIRE FOR ELECTRICAL PURPOSES.

SPECIFICATION forming part of Letters Patent No. 251,970, dated January 3, 1882.

Application filed November 9, 1881. (No specimens.)

*To all whom it may concern:*

Be it known that I, JAMES TAYLOR, of Ansonia, in the county of New Haven and State of Connecticut, have invented a new Improvement in Coating and Insulating Wire for Electrical Purposes; and I do hereby declare the following to be a full, clear, and exact description of the same.

This invention relates to an improvement in preparing wire, copper strips, &c., for electrical purposes, the object being to more perfectly insulate the wire or strip than has heretofore been done; and it consists, essentially, in a coating of benzoin applied either directly to the wire or outside of a fibrous coating first placed upon the wire, as more fully hereinafter described. The benzoin with which the insulation or coating is to be made is first dissolved in alcohol in proportions to bring the benzoin into such condition as to be readily applied with a brush or so as to adhere to the wire when drawn through it.

First. To insulate bare wire which is to be wound or braided with a fibrous material, I arrange a bath, which will contain the benzoin, near the machine which is to apply the fibrous material. This machine may be a common winder or braider. The wire is drawn through the bath, thence immediately through the machine which applies the fibrous material, so that the fibrous material will come into contact with the coated surface before the benzoin coating shall have hardened, whereby the fibrous material adheres to the coating and is firmly fixed upon the surface of the wire. The benzoin not only makes a most perfect insulator, but serves as the best cement to secure the covering upon the wire.

Second. Insulating wire which has been covered with fibrous material not only to insulate the wire, but to make a perfect water-proof covering: The wire is wound or braided with fibrous material in the usual manner, and then passed through a bath of benzoin. The benzoin fills the interstices of the braiding and coats the surface, so as to render it water-proof and make the most perfect insulator.

Third. To coat wire which has been covered with fibrous material by braiding or winding,

and in which the covering has been filled with 50 paraffine: In this third use the wire is covered, the covering filled with paraffine and polished in the usual manner; then it is drawn through a bath of benzoin.

In all the processes of applying the benzoin 55 to the outside the movement of the wire as it passes from one drum to another should be so slow as to allow the alcohol in which the benzoin is dissolved to evaporate before it reaches the drum on which it is coiled after coming 60 from the bath.

The benzoin coating is improved by applying a sponge saturated with the benzoin to the surface as it passes toward the drum, which distributes the benzoin evenly over the surface. 65

In the use of benzoin as a final coating for wire which has been covered and the covering saturated with paraffine the benzoin preparation possesses an advantage over other known coatings from the fact that neither the benzoin 70 or alcohol in which it is dissolved is a solvent of paraffine or any ingredients—as beeswax—with which paraffine is mixed. Hence the benzoin retains upon the outside all its insulating properties, is flexible, permits the wire to be bent 75 without disturbing the coating, and does not in any degree affect the covering which lies between it and the wire, each of the parts retaining in themselves their own independent properties. 80

For some uses the simple coating of the surface of the wire with the benzoin is all the insulation that will be necessary, because the benzoin forms a coating upon the outside of the wire so hard as not to be easily broken, and 85 which is a most perfect insulator, but where the wire is to be exposed to any considerable extent the fibrous covering is desirable.

It will be understood that the same benzoin coating is used in the preparation of strips of 90 copper—that is to say, the benzoin is applied directly to the surface of the strip, and the fabric, if required, is laid upon the strip while the benzoin coating is in an adhesive condition, so as to secure the strip to the copper in 95 the most perfect manner, at the same time insulating the strip.

I do not wish to be understood as broadly

claiming insulating copper wire or strips by coating directly upon the surface of the wire or strip, or by a coating outside the covering, as such I am aware is not new; but

5. What I do claim is—

1. Wire or copper strips for electrical purposes, having the surface coated with benzoin, substantially as described.

2. Copper wire or strips for electrical purposes first coated with benzoin, then with a fibrous covering applied to the benzoin-coated surface while the benzoin is in an adhesive state, substantially as described.

3. Copper wire or strips for electrical pur-

poses first coated with a fibrous material, then 15 a fibrous covering coated with benzoin, substantially as described.

4. Copper wire or strips for electrical purposes first coated with a fibrous material, the fibrous material filled with paraffine, or a composition of which paraffine forms the base, then 20 finally coated with benzoin, substantially as and for the purpose described.

JAMES TAYLOR.

Witnesses:

JOSIAH H. WHITING,  
JOHN D. BALLOU.